



compositions (A, B, and C) of the invention include the following:

TABLE I  
Sulfate bath

(1):

|                                           |                                               |
|-------------------------------------------|-----------------------------------------------|
| $\text{CuSO}_4 \cdot 5\text{H}_2\text{O}$ | 150-300 g./l. (preferably about 220 g./l.).   |
| $\text{H}_2\text{SO}_4$                   | 10-100 g./l. (preferably about 60 g./l.).     |
| $\text{Cl}^-$                             | 5-150 mg./l. (preferably about 20-80 mg./l.). |

Fluoborate bath

(2):

|                            |                                               |
|----------------------------|-----------------------------------------------|
| $\text{Cu}(\text{BF}_4)_2$ | 100-600 g./l. (preferably about 224 g./l.).   |
| $\text{HBF}_4$             | 1-60 g./l. (preferably about 3.5 g./l.).      |
| $\text{H}_3\text{BO}_3$    | 0-30 g./l. (preferably about 15 g./l.).       |
| $\text{Cl}^-$              | 5-150 mg./l. (preferably about 20-80 mg./l.). |

The basis metals which may be electroplated in accordance with the process of this invention may include ferrous metals, such as steel, iron, etc., bearing a surface layer of nickel or cyanide copper; zinc and its alloys including zinc-base die-cast articles bearing a surface layer of cyanide copper or pyrophosphate copper; nickel, including nickel alloys with other metals such as cobalt; aluminum, including its alloys, after suitable pretreatment, etc.

After the deposition of the bright leveled copper deposit of this invention, generally a bright nickel deposit and a chromium deposit (which may be microporous or microcracked) may be applied. The bright acid copper deposit of this invention contributes to the appearance and performance of the composite coating because of its very high rate of leveling, its excellent pore-filling capacity, its high luster, good ductility and low internal stress. It improves corrosion resistance and permits economy in nickel use.

Because of its strong leveling properties, its very good performance at high current densities, and its very good mechanical properties (especially good ductility and low stress) the bright acid copper electrodeposits of this invention may be used for industrial applications such as electroforming, the plating of memory drums, printing rolls, etc. The process gives very good results also for the plating of non-conducting materials, such as plastics, after the usual pretreatment.

The plating conditions for electrodeposition from the aforementioned baths may, for example, include temperatures of 10° C.-60° C. (preferably 20° C.-40° C.); pH (electrometric) of less than about 2.5; and a cathode current density of .1-50.0 amperes per square decimeter (asd).

Typical average current densities may be 2-20 asd for the sulfate bath and about 4-40 asd for the fluoborate bath. Air agitation, volume agitation, or mechanical agitation may increase the effective current density ranges and enhance the uniformity of the copper deposit.

In accordance with certain of its aspects, this invention relates to novel compositions and to a process for electrodepositing bright, strongly leveled, ductile copper from an aqueous acidic copper plating bath containing chloride ions and at least one member independently selected from each of the following groups:

(A) a polysulfide compound of the formula



(B) a heterocyclic sulfur compound containing the grouping



5

and/or tautomers thereof, where the nitrogen atom and the two carbon atoms are part of a heterocyclic ring; and

(C) a polyether containing at least 5 ether oxygen atoms per molecule;

wherein R is independently a divalent aliphatic or aromatic non-heterocyclic group of 1-10 carbon atoms; R' is hydrogen, a metal cation, a monovalent aliphatic or aromatic group of 1-20 carbon atoms, or the groups  $-\text{R}-\text{SO}_3\text{M}$  or  $-\text{R}-(\text{S})_q-\text{RSO}_3\text{M}$  wherein q is an integer 2-5; M is a cation; Z is 0 or 1, R'' is hydrogen, a metal ion or one of the groups



25

wherein R''' is hydrogen, an alkyl group of 1-6 carbon atoms, aryl, alkaryl or aralkyl group.

Sulfide compounds wherein n is an integer 2-4 are preferred. R may be a divalent hydrocarbon group (including such hydrocarbon groups containing inert substituents such as hydroxyl, alkoxy, polyoxyalkylene, halogen, etc.) of 1-10 carbon atoms such as an alkylene group of 1-10 carbon atoms (i.e.  $-\text{CH}_2-$ ,  $-\text{CH}_2\text{CH}_2-$ ,  $-(\text{CH}_2)_3-$ ,  $-(\text{CH}_2)_5-$ , and, in general,  $-(\text{CH}_2)_p-$  wherein p is an integer 1-10. R may be a divalent non-heterocyclic group of 1-10 carbon atoms containing 1-3 oxygen, 1-3 sulfur, or 1-3 nitrogen atoms (such as



50 etc.).

In the compound



55 R' may be a hydrocarbon radical preferably selected from the group consisting of alkyl, alkenyl, alkynyl, cycloalkyl, aralkyl, aryl, alkaryl, including such radicals when inertly substituted. When R' is alkyl, it may typically be

60 straight chain alkyl or branched alkyl, including methyl, ethyl, n-propyl, isopropyl, n-butyl, isobutyl, sec-butyl, tert-butyl, n-amyl, neopentyl, isoamyl, n-hexyl, isohexyl, heptyls, octyls, decyls, dodecyls, etc. Preferred alkyl includes lower alkyl, i.e. having less than about 8 carbon atoms, i.e. octyls and lower. When R' is alkenyl, it may typically be vinyl, allyl, methallyl, buten-1-yl, buten-2-yl, butyn-3-yl, penten-1-yl, hexenyl, heptenyl, octenyl, decenyl, dodecenyl, tetra-decenyl, octadecenyl, etc. When R' is alkynyl, it may typically be ethynyl, propargyl, butynyl, etc. When R' is cycloalkyl, it may typically be cyclopentyl, cyclohexyl, cycloheptyl, cyclooctyl, etc. When R' is aralkyl, it may typically be tolyl, xylyl, p-ethylphenyl, p-nonylphenyl, etc. R' may be inertly substituted, e.g. may bear a nonreactive substituent such as alkyl, aryl, cyclo-

70 alkyl, aralkyl, alkaryl, alkenyl, ether, etc.

Polysulfide compounds of the Formula A may typically be prepared by the reaction of an alkali metal salt of a hydrosulfide and a sultone according to the reaction:



wherein R, R', M, and n are as previously defined.

Specific illustrative reactions may include the following 10 reactions wherein all unsubstituted carbon atoms are attached to hydrogen atoms:



Other preparative reactions which may be used to produce the sulfide compounds employed according to the invention include the direct sulfonation of an organo polysulfide (i.e. direct sulfonation of diphenyl disulfide, ditolyl disulfide, etc.). The polysulfide compounds also may be prepared by the reaction of epichlorohydrin and an alkali metal bisulfite followed by reaction with a polysulfide (such as Na<sub>2</sub>S<sub>2</sub>, R'SNa, wherein R' is as previously defined).

Other preparative reactions may include the following:

- (a)  $\text{SCl}_2 + 2\text{NaS}(\text{CH}_2)_3\text{SO}_3\text{Na} \rightarrow \text{NaO}_3\text{S}(\text{CH}_2)_3\text{S}-\text{S}-\text{S}-(\text{CH}_2)_3\text{SO}_3\text{Na}$
- (b)  $\text{S}_2\text{Cl}_2 + 2\text{NaS}(\text{CH}_2)_3\text{SO}_3\text{Na} \rightarrow \text{NaO}_3\text{S}(\text{CH}_2)_3\text{S}-\text{S}-\text{S}-(\text{CH}_2)_3\text{SO}_3\text{Na}$
- (c)  $\text{ClCH}_2\text{CH}_2\text{Cl} + 2\text{NaSS}(\text{CH}_2)_3\text{SO}_3\text{Na} \rightarrow \text{NaO}_3\text{S}(\text{CH}_2)_3\text{SSCH}_2\text{CH}_2\text{SS}(\text{CH}_2)_3\text{Na}$
- (d)  $\text{ClCH}_2\text{CH}_2\text{Cl} + \text{NaSS}(\text{CH}_2)_3\text{SO}_3\text{Na} + \text{NaS}(\text{CH}_2)_3\text{SO}_3\text{Na} \rightarrow \text{NaO}_3\text{S}(\text{CH}_2)_3\text{SSCH}_2\text{CH}_2\text{S}(\text{CH}_2)_3\text{SO}_3\text{Na}$

Typical polysulfide compounds which may be employed according to the invention include the following compounds which are summarized in Table II. In the formula

M represents a sodium cation and R, R', and N are as indicated in Table II.

TABLE II  
[Sulfonated polysulfide cooperating brighteners of the Formula



| Additive    | R'                                                                                  | n R                                     |
|-------------|-------------------------------------------------------------------------------------|-----------------------------------------|
| 10 A-1....  |    | 2 (CH <sub>2</sub> ) <sub>3</sub>       |
| 15 A-2....  |    | 2 (CH <sub>2</sub> ) <sub>3</sub>       |
| 20 A-3....  |    | 2 (CH <sub>2</sub> ) <sub>3</sub>       |
| 25 A-4....  |    | 2 (CH <sub>2</sub> ) <sub>3</sub>       |
| 30 A-5....  |   | 2 (CH <sub>2</sub> ) <sub>3</sub>       |
| 35 A-6....  |  | 2 (CH <sub>2</sub> ) <sub>3</sub>       |
| 40 A-7....  |  | 2                                       |
| 45 A-8....  |  | 2 (CH <sub>2</sub> ) <sub>3</sub>       |
| 50 A-9....  |  | 2 (CH <sub>2</sub> ) <sub>3</sub>       |
| A-10....    |  | 2 (CH <sub>2</sub> ) <sub>4</sub>       |
| A-11....    |  | 4 (CH <sub>2</sub> ) <sub>3</sub>       |
| A-12....    |  | 2 (CH <sub>2</sub> ) <sub>3</sub>       |
| A-13....    |  | 2 (CH <sub>2</sub> ) <sub>3</sub>       |
| A-14....    |  | 2 (CH <sub>2</sub> ) <sub>3</sub>       |
| A-15....    |  | 2 (CH <sub>2</sub> ) <sub>3</sub>       |
| A-16....    |  | 2 (CH <sub>2</sub> ) <sub>3</sub>       |
| A-17....    |  | 2 (CH <sub>2</sub> ) <sub>3</sub>       |
| A-18....    |  | 2 (CH <sub>2</sub> ) <sub>3</sub>       |
| A-19....    |  | 2 (CH <sub>2</sub> ) <sub>3</sub>       |
| A-20....    |  | 2 (CH <sub>2</sub> ) <sub>3</sub>       |
| 60 A-21.... |  | 2 (CH <sub>2</sub> ) <sub>3</sub>       |
| 65 A-22.... |  | 2 CH <sub>2</sub> CH(OH)CH <sub>3</sub> |

The R'-(S)<sub>n</sub>Na compound may be prepared by the reaction of R'SNa with sulfur if R' is an aromatic group (compounds A-1, A-2, A-3, A-4, A-5, A-20). A typical procedure is: To a methanol solution (150 ml.) containing sodium methoxide (0.1 m.) is added the R'SNa (0.1 m.) compound. The mixture is stirred at room temperature until the compound has dissolved. Sulfur powder (0.1 gram-equivalent) is added and the mixture stirred

until all the sulfur is dissolved. Propanesultone (0.12 mole) is added to the stirred solution. Stirring is continued for 30 minutes, during which time a solid precipitates from the solution. Acetone (250 ml.) is then added to give additional solid, which is then filtered, washed with acetone, and dried.

Aliphatic  $R'(S)_nNa$  compounds are prepared by reaction of  $R'Q$  with  $Na_2S_m$ , where  $Q$  is  $Cl$ ,  $Br$ ,  $I$ ,  $-\text{OSO}_2\text{C}_6\text{H}_5$ ,  $-\text{OSO}_2\text{C}_6\text{H}_4\cdot\text{CH}_3$ ,  $-\text{OSO}_2\text{CH}_3$  (e.g. compounds A-17, A-18, A-19). A typical procedure is: To a stirred methanol solution (150 ml.) containing sodium disulfide (0.1 m.) is added dropwise a solution of  $R'Q$  (0.1 m.) in methanol (50 ml.) at room temperature. The reaction is slightly exothermic. After the addition is completed the mixture is stirred for 30 minutes. Propane sultone (0.12 m.), which may be dissolved in methanol (50 ml.), is added to the stirred mixture. During the addition of propane sultone a white solid usually precipitates from the solution. The mixture may be heated and stirred at  $65^\circ\text{C}$ . for 30 minutes and then cooled. Acetone is added and the solid is filtered and dried.

Compounds of the type of A-9, A-10, A-11, A-12 are prepared by the reaction of an alkali metal polysulfide ( $Na_2S_2$ ,  $Na_2S_4$ , etc.) with a sultone.

Compounds of the type of A-13, A-14, A-15, A-16 are prepared according to the reaction sequence:



Instead of sultones, haloalkane sulfonates, including e.g.  $\text{ClCH}_2\text{CHOHCH}_2\text{SO}_3\text{Na}$  (prepared by reaction of epichlorohydrin with sodium bisulfite), and in general compounds of the type  $\text{QSRO}_3\text{M}$ , may be used.

Some polysulfide compounds may also be prepared by the direct sulfonation of an organic polysulfide (e.g. A-7; or A-21 by sulfonation of A-20).

Symmetrical disulfides may be prepared by careful oxidation of compounds of the type  $\text{HRSO}_3\text{Na}$ .

It is sometimes advantageous to prepare aqueous stock solutions of the sulfonated polysulfides containing small amounts of copper sulfate and/or sulfuric acid. Some precipitation may occur which is eliminated by filtration.

The sulfide compounds of the invention may be present in the copper bath in effective amounts of about 0.001 g./l.-1.0 g./l., preferably 0.005 g./l.-0.2 g./l.-0.2 g./l.

The heterocyclic sulfur-containing cooperating additives of this invention contain the grouping:

a heterocyclic sulfur compound containing the grouping



and/or tautomers thereof, where the nitrogen atom and the two carbon atoms are part of a heterocyclic ring wherein  $Z$  is  $O$  or  $1$ ; and  $R''$  is hydrogen, a metal ion or one of the groups



wherein  $R'''$  is hydrogen, an alkyl group of 1-6 carbon atoms, aryl, alkaryl or aralkyl group.

Alternatively, the heterocyclic sulfur compound is of the formula



and/or tautomers thereof,  $N$ -oxides of said compound, isothiourea derivatives, isothioamide derivatives and di-

thiocarbamate derivatives thereof where  $R_1$  is hydrogen, a metal cation, or the groups



wherein  $R''$  is hydrogen, an alkyl group of 1-6 carbon atoms, aryl, alkaryl, or aralkyl;  $X$  is  $-\text{CR''}=\text{}$  or  $-\text{CR''}_2-$  and  $Y$  is a divalent organogroup of 2 to 16 carbon atoms which forms 1 or more 5 through 7 membered cyclic ring structure or structures with the group



wherein  $X$  and  $R_1$  are as hereinbefore defined.

Typical parent substances are: 2-mercaptop pyridine, 2-mercaptop quinoline, 1- or 4-mercaptop isoquinoline; their  $N$ -oxides; alkyl, hydroxy, alkoxy, mercapto derivatives of these compounds derived by substitution on the ring carbon atoms; isothioureas, isothioamides and their salts with acids, dithiocarbamates derived by substitution on the bivalent sulfur atom. Among the heteroaliphatic ring compounds thiocaprolactam gives especially good results.

The mercapto compounds may be dissolved before addition to the copper bath in water containing equivalent amounts of alkali hydroxides, in dilute acids or in suitable organic solvents, e.g. alcohols. The isothiourea, isothioamide, dithiocarbamate derivatives are dissolved in water, dilute acids or in suitable solvents such as alcohols, but not in alkali hydroxides as they may decompose therein.

The function of the heterocyclic compounds of group (B) is to produce, in conjunction with the sulfonated polysulfides of group (A) and the polyethers of group (C), leveling and to increase the brightness of the deposits obtained, especially in the low and medium current density range.

The heterocyclic compounds of formula group (B) may be employed in effective amounts, typically 0.1-50 mg./l. and preferably 0.5-20 mg./l. of total aqueous bath composition. Typical heterocyclic group (B) compounds which may be employed according to the invention are given in Table III.

TABLE III.—HETEROCYCLIC COMPOUNDS (B)

| B    | Formula | Name                                                     |
|------|---------|----------------------------------------------------------|
| 1... |         | 2-mercaptopyridine (2-pyridinethiol).                    |
| 2... |         | 2-S-pyridyl isothiouronium chloride.                     |
| 3... |         | 2-mercaptopyridine-n-oxide (1-hydroxy-2-pyridinethione). |
| 4... |         | 2-S-pyridyl isothiouronium chloride N-oxide.             |
| 5... |         | 2-mercaptop-4-methylpyridine.                            |

TABLE III—Continued

| B     | Formula | Name                                                  |
|-------|---------|-------------------------------------------------------|
| 6...  |         | 4-methyl-2-S-pyridyl isothiouronium chloride.         |
| 7...  |         | 2-mercaptop-4-methylpyridine-N-oxide.                 |
| 8...  |         | 4-methyl-2-S-pyridyl isothiouronium chloride N-oxide. |
| 9...  |         | 2-mercaptop-6-methylpyridine.                         |
| 10... |         | 6-methyl-2-S-pyridyl isothiouronium chloride.         |
| 11... |         | 2-mercaptop-6-methylpyridine-N-oxide.                 |
| 12... |         | 6-methyl-2-S-pyridyl isothiouronium chloride N-oxide. |
| 13... |         | 2-mercatoquinaline.                                   |
| 14... |         | 2-S-quinolyl isothiouronium chloride.                 |
| 15... |         | 2-mercatoquinaline N-oxide.                           |
| 16... |         | 2-S-quinolyl isothiouronium chloride N-oxide.         |

TABLE III—Continued

| B     | Formula | Name                                                                   |
|-------|---------|------------------------------------------------------------------------|
| 17... |         | 2-mercaptop-6-hydroxypyridine.                                         |
| 5     |         | 6-hydroxy-2-S-pyridyl isothiouronium chloride.                         |
| 10    |         | 2,6-dimercaptopyridine.                                                |
| 15    |         | 2,6-SS-pyridyl bis-isothiouronium chloride.                            |
| 20    |         | Thiocaprolactam (2-thioxohexamethylene imine).                         |
| 25    |         | 2-S-pyridyl-N-diethyl dithiocarbamate.                                 |
| 30    |         |                                                                        |
| 35    |         |                                                                        |
| 40    |         |                                                                        |
| 45    |         |                                                                        |
| 50    |         |                                                                        |
| 55    |         |                                                                        |
| 60    |         | $R'''-O-Z$                                                             |
| 65    |         | $R'''-S-Z$                                                             |
| 70    |         | $R''' \begin{array}{c} \diagup \\ N-Z \\ \diagdown \\ R'' \end{array}$ |
| 75    |         | $R'''-N \begin{array}{c} \diagup \\ Z \\ \diagdown \end{array}$        |
|       |         | $R''''(OZ)_m$                                                          |
|       |         | $R''''(SZ)_m$                                                          |

The heterocyclic cooperating additives of Table III are available commercially. The heterocyclic compounds of Table III (with the exception of B-21) are generally prepared from the corresponding halogen compounds, e.g. 2-chloropyridine either by direct reaction with alkali metal hydrosulfide or more frequently just with thiourea joining the respective isothiouronium compounds, which may be converted by alkaline hydrolysis into the corresponding mercapto compounds. B-22 was synthesized by reaction of 2-chloropyridine with sodium diethylthiocarbamate.

Polyethers which may be used according to the process of the invention may have at least 5 ether oxygen atoms and include polyethers of the formulae:

55

60

 $R'''-O-Z$ 

65

 $R'''-S-Z$  $R''' \begin{array}{c} \diagup \\ N-Z \\ \diagdown \\ R'' \end{array}$ 

70

 $R'''-N \begin{array}{c} \diagup \\ Z \\ \diagdown \end{array}$ 

75

 $R''''(OZ)_m$  $R''''(SZ)_m$



where  $R'''$  is a monovalent radical such as  $H$ , alkyl, alkenyl, alkynyl, alkylaryl, arylalkyl or a heterocyclic radical; and  $R'''$  is a  $m$ -valent aliphatic, aromatic or heterocyclic radical;  $n=2$  to 100; and



where  $u$  and  $v=0$  to 4, but at least one of  $u$  or  $v$  must be greater than zero;  $r+s=6$  to 200,000;  $r=0$  when  $u=0$ ;  $s=0$  when  $v=0$ ; and  $T=H$ , alkyl, benzyl,  $-SO_3M$ ,  $-C_uH_{2u}SO_3M$ ,  $-PO_3H_2$ , or  $C_uH_{2u}NHR'''$ .

Suitable polyethers which may be used according to the invention include polyethers set forth in Table IV. The polyether additives may be employed in effective amounts, typically 0.005-10.0 g./l. and preferably 0.1-1.0 g./l. of total aqueous bath compositions.

TABLE IV.—COOPERATING POLYETHERS

| Additive |                                                                                                                                                                                                                                                                                        |
|----------|----------------------------------------------------------------------------------------------------------------------------------------------------------------------------------------------------------------------------------------------------------------------------------------|
| C-1..... | $CH_3 \begin{array}{c} CH_3 \\   \\ CH_3-CH-CH_2-C-C=C-C=CH_2-CH-CH_3 \\   \quad   \\ O \quad O \\ \left[ \begin{array}{c} CH_2 \\   \\ CH_2 \end{array} \right]_m \left[ \begin{array}{c} CH_2 \\   \\ CH_2 \end{array} \right]_n \\   \quad   \\ O \quad O \\ H \quad H \end{array}$ |
|          | $m+n=30$                                                                                                                                                                                                                                                                               |
| C-2..... | Formula C-1 wherein $m+n=15$ .                                                                                                                                                                                                                                                         |
| C-3..... | Formula C-1 wherein $m+n=10$ .                                                                                                                                                                                                                                                         |
| C-4..... | $CH_3 \begin{array}{c} CH_3 \\   \\ CH_3-C-CH_2-C- \\   \quad   \\ CH_3 \quad CH_3 \end{array} \begin{array}{c} \text{C}_6\text{H}_4 \\   \\ O-(CH_2CH_2O)_xH \end{array}$                                                                                                             |
|          | $x=9-10$                                                                                                                                                                                                                                                                               |
| C-5..... | Formula C-4 wherein $x=30$ .                                                                                                                                                                                                                                                           |
| C-6..... | Formula C-4 wherein $x=40$ .                                                                                                                                                                                                                                                           |
| C-7..... | $C_9H_{15} \begin{array}{c} \text{C}_6\text{H}_4 \\   \\ O-(CH_2CH_2O)_nH \end{array}$                                                                                                                                                                                                 |
| C-8..... | $n-C_{12}H_{25}O(CH_2CH_2O)_nH$                                                                                                                                                                                                                                                        |
| C-9..... | $n-C_xH_{2x} \begin{array}{c} H \\   \\ C-CH_3 \\   \\ N-(CH_2CH_2O)_yH \\   \\ (CH_2CH_2O)_zH \end{array}$                                                                                                                                                                            |
|          | $x=9-12, y+z=15$                                                                                                                                                                                                                                                                       |
| C-10.... | $H(C_2H_4O)_x(C_2H_4O)_y \begin{array}{c} (C_2H_4O)_z(C_2H_4O)_wH \\   \\ NCH_2CH_2N \\   \\ H(C_2H_4O)_x(C_2H_4O)_yH \end{array}$                                                                                                                                                     |
|          | wherein $x$ is about 3 and $y$ is about 3-4                                                                                                                                                                                                                                            |
| C-11.... | $HO(C_2H_4O)_zH$<br>wherein $z$ is about 13                                                                                                                                                                                                                                            |
| C-12.... | $HO(C_2H_4O)_zH$<br>wherein $z$ is about 33                                                                                                                                                                                                                                            |
| C-13.... | $HO(C_2H_4O)_zH$<br>wherein $z$ is about 6-7                                                                                                                                                                                                                                           |
| C-14.... | $HO(C_2H_4O)_zH$<br>wherein $z$ is about 12                                                                                                                                                                                                                                            |

12  
TABLE IV—Continued

| Additive |                                                                                                                                                                                                                                                                                                                                                                                                                                                                               |
|----------|-------------------------------------------------------------------------------------------------------------------------------------------------------------------------------------------------------------------------------------------------------------------------------------------------------------------------------------------------------------------------------------------------------------------------------------------------------------------------------|
| 5        | $C-15.... \begin{array}{c} CH_3 \quad CH_3 \\   \quad   \\ CH_3-CH_2-C-CH_2-CH_2-C-CH_2-CH_3 \\   \quad   \quad   \quad   \\ O \quad O \quad O \quad O \\ \left[ \begin{array}{c} CH_2 \\   \\ CH_2 \end{array} \right]_m \left[ \begin{array}{c} CH_2 \\   \\ CH_2 \end{array} \right]_n \\   \quad   \quad   \quad   \\ CHCH_3 \quad CH_2 \quad CHCH_3 \quad CH_2 \\   \quad   \quad   \quad   \\ O \quad O \quad O \quad O \\ H \quad H \quad H \quad H \end{array}$       |
| 10       |                                                                                                                                                                                                                                                                                                                                                                                                                                                                               |
| 15       |                                                                                                                                                                                                                                                                                                                                                                                                                                                                               |
| 20       | $C-16.... \begin{array}{c} CH_3 \quad CH_3 \\   \quad   \\ CH_3-CH_2-CH_2-C-CH_2-CH_3 \\   \quad   \quad   \quad   \\ O \quad O \quad O \quad O \\ \left[ \begin{array}{c} CH_2 \\   \\ CH_2 \end{array} \right]_m \left[ \begin{array}{c} CH_2 \\   \\ CH_2 \end{array} \right]_n \\   \quad   \quad   \quad   \\ CHCH_3 \quad CH_2 \quad CHCH_3 \quad CH_2 \\   \quad   \quad   \quad   \\ O \quad O \quad O \quad O \\ H \quad H \quad H \quad H \end{array}$              |
| 25       |                                                                                                                                                                                                                                                                                                                                                                                                                                                                               |
| 30       |                                                                                                                                                                                                                                                                                                                                                                                                                                                                               |
| 35       | $C-17.... C_{12}H_{25}S(CH_2CH_2O)_nH$                                                                                                                                                                                                                                                                                                                                                                                                                                        |
| 40       | $C-18.... \begin{array}{c} H \quad H \\   \quad   \\ H_2N-C-CH_2-\left( \begin{array}{c} O \\   \\ CH_2-C \\   \\ CH_2 \end{array} \right)_pNH_2 \\   \quad   \\ CH_3 \quad CH_3 \end{array}$                                                                                                                                                                                                                                                                                 |
|          | wherein $p$ is about 5-6.                                                                                                                                                                                                                                                                                                                                                                                                                                                     |
| 45       | $C-19.... \begin{array}{c} H \quad H \\   \quad   \\ H_2N-C-CH_2-\left( \begin{array}{c} O \\   \\ CH_2-C \\   \\ CH_2 \end{array} \right)_pNH_2 \\   \quad   \\ CH_3 \quad CH_3 \end{array}$                                                                                                                                                                                                                                                                                 |
|          | wherein $p$ is about 18.                                                                                                                                                                                                                                                                                                                                                                                                                                                      |
| 50       | $C-20.... CH_3(CH_2)_nCHCH_3$<br>$O(C_2H_4O)_n(C_2H_4O)_mH$                                                                                                                                                                                                                                                                                                                                                                                                                   |
| 55       | $C-21.... CH_3(CH_2)_nO(C_2H_4O)_m(C_2H_4O)_pH$<br>$C-22.... CH_3(CH_2)_nO(C_2H_4O)_m(C_2H_4O)_pH$<br>$C-23.... HO(C_2H_4O)_nO(CH_2)_mO(C_2H_4O)_pH$                                                                                                                                                                                                                                                                                                                          |
| 60       | $C-24.... H(O(C_2H_4O)_nCH_2C-CH_2-CH-CH_2CH_2N(C_2H_4O)_pH$<br>$H(OH_2C)_nCH_2C-CH_2-CH-CH_2CH_2N(C_2H_4O)_pH$<br>$C-25.... HO(C_2H_4O)_nH$<br>$wherein z is about 136 (M.w. is about 6,000)$<br>$C-26.... HO(C_2H_4O)_nH$<br>$wherein z is about 454 (M.w. is about 20,000)$<br>$C-27.... HO(C_2H_4O)_nH$<br>$wherein z is about 4,540 (M.w. is about 200,000)$                                                                                                             |
| 65       | <p>The chloride ion content of the aqueous copper plating bath compositions of the invention may be at least about 0.5 mg./l. and typically from 1.0 mg./l. to 500 mg./l. of aqueous copper plating bath. Good results may be obtained using a chloride ion concentration of from about 3 mg./l. to 100 mg./l. of aqueous copper plating bath composition, and preferably a chloride ion concentration of from 20 mg./l. to 80 mg./l. of aqueous copper plating solution.</p> |
| 70       |                                                                                                                                                                                                                                                                                                                                                                                                                                                                               |
| 75       |                                                                                                                                                                                                                                                                                                                                                                                                                                                                               |

Other optional additives used were the following dispersing agents:

measured as "poor," "fair," "good," and "very good" as follows:

TABLE V

| Additives                                                                                                                                              |
|--------------------------------------------------------------------------------------------------------------------------------------------------------|
| D-1.....                                                                                                                                               |
| CH <sub>2</sub> -                                                                                                                                      |
| D-2.....                                                                                                                                               |
| NaO <sub>2</sub> S-                                                                                                                                    |
| D-3.....                                                                                                                                               |
|                                                                                                                                                        |
| where n=3 to 6                                                                                                                                         |
| D-4.....                                                                                                                                               |
|                                                                                                                                                        |
| n+m=1-2 and preferably n=0 when m=1;                                                                                                                   |
| D-5.....                                                                                                                                               |
|                                                                                                                                                        |
| wherein each n is an integer 4-12 (preferably 4-8) and each M <sub>1</sub> and M <sub>2</sub> an alkali metal (preferably Na or K) or a hydrogen atom. |

The following examples are set forth for the purpose of providing those skilled-in-the-art with a better understanding of this invention, and the invention is not to be construed as limited to such examples.

In these examples the aqueous copper plating bath contains unless noted otherwise:

|                                     | G./L. |
|-------------------------------------|-------|
| CuSO <sub>4</sub> 5H <sub>2</sub> O | 220   |
| H <sub>2</sub> SO <sub>4</sub>      | 60    |
| Chloride ion                        | 0.06  |

The plating experiments were performed in a Hull Cell containing 250 ml. of this acid copper sulfate bath. The Hull Cell allows one to observe the appearance of the deposit over a wide current density range. In order to judge the degree of leveling the polished brass panels used for these plating tests were scratched with 4/0 emery polishing paper over a horizontal band of about 10 mm. width. The plating temperature used in these experiments was the ambient room temperature (24-30°C.), unless otherwise stated. The total current was 2 amperes and the plating time 10 minutes. Air agitation or mechanical agitation with an oscillating paddle was used as specified in Table VI. The sulfonated polysulfide compounds used are described in Table II, the heterocyclic sulfur compounds in Table III, and the polyethers in Table IV.

For convenience, the results shown in Table VI are classified according to (1) the width of the lustrous current density range (semi-bright to bright) and according to (2) the degree of leveling under the indicated experimental conditions (i.e. a 250 ml. Hull Cell, 2 amperes current, and a ten minute plating time on a metal strip having a band uniformly scratched with 4/0 grit emery paper).

Each property in groups (1) and (2) is independently

|    | Property (1)                                                                   | Property (2)                                                                                                               |
|----|--------------------------------------------------------------------------------|----------------------------------------------------------------------------------------------------------------------------|
|    | Rating... Width of lustrous current density range                              | Rating... Degree of leveling.                                                                                              |
| 45 | Poor..... Less than one half of length of test panel.                          | Poor.... No visual change in original roughness of scratched band.                                                         |
|    | Fair..... More than one half and less than two thirds of length of test panel. | Fair..... Noticeable decrease in roughness, but scratches still visible.                                                   |
|    | Good.... More than two thirds but less than entire length of test panel.       | Good... Roughness decreased and portions of scratches completely level.                                                    |
| 50 | Very good. Entire length of test panel is lustrous.                            | Very good. Scratches on the portion of the panel having a current density greater than 2.5 asd. are practically invisible. |

55 The combination of the panel ratings given with respect to width of lustrous current density range and degree of leveling determine the final classification set forth in the "Results" column of Table VI according to the following:

|    |                 |                                                                                                                                                          |
|----|-----------------|----------------------------------------------------------------------------------------------------------------------------------------------------------|
| 60 | Result          | Definition                                                                                                                                               |
|    | Excellent ----- | Very good leveling and very good bright current density range.                                                                                           |
| 65 | Very good ----- | Very good leveling and good bright current density range.                                                                                                |
|    | Good -----      | Good to very good leveling and good to very good semi-bright current density range or: good leveling and good to very good bright current density range. |
| 70 | Poor -----      | Poor leveling and/or poor lustrous current density range.                                                                                                |
|    | Fair -----      | All intermediate panels not otherwise classified.                                                                                                        |

TABLE VI

| Example number | Additive       | Amounts, g./l. | Type of agitation          | Results             |
|----------------|----------------|----------------|----------------------------|---------------------|
| 1              | {A-1<br>[C-1   | 0.02<br>1.0    | Air.....<br>Air.....       | Poor.<br>Do.        |
| 2              | {A-1<br>[B-3   | 0.02<br>0.006  | Air.....<br>Air.....       | Very good.<br>Do.   |
| 3              | {C-1<br>[B-11  | 1.0<br>0.004   | Air.....<br>Air.....       | Do.<br>Excellent.   |
| 4              | {A-1<br>[B-12  | 0.02<br>0.003  | Air.....<br>Air.....       | Do.<br>Excellent.   |
| 5              | {A-1<br>[C-7   | 0.02<br>1.0    | Mechanical.....<br>do..... | Poor.<br>Do.        |
| 6              | {A-1<br>[B-5   | 0.02<br>0.002  | Mechanical.....<br>do..... | Excellent.<br>Do.   |
| 7              | {A-1<br>[C-8   | 0.02<br>1.0    | Mechanical.....<br>do..... | Poor.<br>Do.        |
| 8              | {C-8<br>[B-16  | 0.02<br>0.002  | Mechanical.....<br>do..... | Excellent.<br>Do.   |
| 9              | {A-2<br>[C-13  | 0.02<br>1.0    | Air.....<br>Air.....       | Poor.<br>Do.        |
| 10             | {A-2<br>[C-13  | 0.02<br>1.0    | Air.....<br>Air.....       | Very good.<br>Do.   |
| 11             | {A-6<br>[C-1   | 0.02<br>1.0    | Air.....<br>Air.....       | Poor.<br>Do.        |
| 12             | {A-6<br>[B-1   | 0.002<br>0.003 | Air.....<br>Air.....       | Good.<br>Do.        |
| 13             | {C-1<br>[B-3   | 0.004<br>0.02  | Air.....<br>Air.....       | Do.<br>Very good.   |
| 14             | {A-6<br>[B-13  | 0.02<br>0.002  | Air.....<br>Air.....       | Do.<br>Do.          |
| 15             | {A-9<br>[C-13  | 0.015<br>0.25  | Air.....<br>Air.....       | Poor.<br>Do.        |
| 16             | {A-9<br>[C-13  | 0.015<br>0.25  | Air.....<br>Air.....       | Very good.<br>Do.   |
| 17             | {A-9<br>[C-13  | 0.015<br>0.25  | Air.....<br>Air.....       | Do.<br>Very good.   |
| 18             | {A-9<br>[C-13  | 0.015<br>0.25  | Air.....<br>Air.....       | Poor.<br>Very good. |
| 19             | {A-9<br>[C-22  | 0.003<br>0.015 | Air.....<br>Air.....       | Do.<br>Do.          |
| 20             | {A-9<br>[C-22  | 0.002<br>0.003 | Air.....<br>Air.....       | Poor.<br>Excellent. |
| 21             | {A-9<br>[C-22  | 0.015<br>1.0   | Air.....<br>Air.....       | Do.<br>Very good.   |
| 22             | {A-9<br>[B-12  | 0.015<br>0.003 | Air.....<br>Air.....       | Do.<br>Do.          |
| 23             | {A-9<br>[B-13  | 0.015<br>0.002 | Air.....<br>Air.....       | Do.<br>Do.          |
| 24             | {A-9<br>[C-22  | 0.015<br>1.0   | Air.....<br>Air.....       | Good.<br>Very good. |
| 25             | {A-9<br>[B-14  | 0.015<br>0.020 | Air.....<br>Air.....       | Do.<br>Do.          |
| 26             | {A-9<br>[B-16  | 0.015<br>0.002 | Air.....<br>Air.....       | Excellent.<br>Do.   |
| 27             | {A-9<br>[B-18  | 0.015<br>0.004 | Air.....<br>Air.....       | Do.<br>Do.          |
| 28             | {A-9<br>[B-19  | 0.015<br>0.002 | Air.....<br>Air.....       | Good.<br>Do.        |
| 29             | {A-9<br>[B-20  | 0.015<br>0.010 | Air.....<br>Air.....       | Do.<br>Do.          |
| 30             | {A-9<br>[B-21  | 0.015<br>0.003 | Air.....<br>Air.....       | Excellent.<br>Do.   |
| 31             | {A-9<br>[B-22  | 0.015<br>0.02  | Air.....<br>Air.....       | Do.<br>Do.          |
| 32             | {A-9<br>[C-25  | 0.015<br>0.25  | Air.....<br>Air.....       | Poor.<br>Do.        |
| 33             | {A-9<br>[B-5   | 0.015<br>0.002 | Air.....<br>Air.....       | Excellent.<br>Do.   |
| 34             | {A-9<br>[B-13  | 0.015<br>0.002 | Air.....<br>Air.....       | Poor.<br>Do.        |
| 35             | {A-9<br>[B-11  | 0.015<br>0.004 | Air.....<br>Air.....       | Excellent.<br>Do.   |
| 36             | {A-9<br>[B-13  | 0.015<br>0.002 | Air.....<br>Air.....       | Good.<br>Do.        |
| 37             | {A-9<br>[C-27  | 0.015<br>0.4   | Air.....<br>Air.....       | Poor.<br>Do.        |
| 38             | {A-9<br>[B-5   | 0.015<br>0.002 | Air.....<br>Air.....       | Very good.<br>Do.   |
| 39             | {A-11<br>[C-10 | 0.02<br>1.0    | Air.....<br>Air.....       | Poor.<br>Do.        |

TABLE VI—Continued

| Example number | Additive       | Amounts, g./l. | Type of agitation    | Results                     |                         |
|----------------|----------------|----------------|----------------------|-----------------------------|-------------------------|
| 5              | 40             | {A-11<br>[C-10 | 0.02<br>1.0          | Air.....<br>Air.....        | Good.<br>Do.            |
| 41             | {A-11<br>[B-11 | 0.02<br>0.004  | Air.....<br>Air..... | Good.<br>Do.                |                         |
| 42             | {A-12<br>[C-18 | 0.02<br>1.0    | Air.....<br>Air..... | Poor.<br>Do.                |                         |
| 10             | 43             | {A-12<br>[C-18 | 0.02<br>1.0          | Air.....<br>Air.....        | Good.<br>Do.            |
| 44             | {A-12<br>[B-18 | 0.004<br>0.008 | Air.....<br>Air..... | Good.<br>Do.                |                         |
| 45             | {A-15<br>[C-15 | 0.02<br>1.0    | Air.....<br>Air..... | Poor.<br>Do.                |                         |
| 15             | 46             | {A-15<br>[C-15 | 0.04<br>1.0          | Air.....<br>Air.....        | Very good.<br>Do.       |
| 47             | {A-15<br>[B-1  | 0.02<br>0.002  | Air.....<br>Air..... | Very good.<br>Do.           |                         |
| 20             | 48             | {C-15<br>[B-13 | 0.02<br>0.002        | Air.....<br>Air.....        | Good.<br>Do.            |
| 49             | {A-17<br>[C-21 | 0.02<br>1.0    | Air.....<br>Air..... | Poor.<br>Do.                |                         |
| 50             | {A-17<br>[D-1  | 0.4<br>0.4     | Air.....<br>Air..... | Do.<br>Do.                  |                         |
| 25             | 51             | {A-17<br>[C-21 | 0.02<br>1.0          | Air.....<br>Air.....        | Good but pitted.<br>Do. |
| 52             | {A-17<br>[B-18 | 0.008<br>0.006 | Air.....<br>Air..... | Very good.<br>Do.           |                         |
| 30             | 53             | {C-9<br>[A-18  | 1.0<br>0.02          | Air.....<br>Mechanical..... | Do.<br>Good.            |
| 54             | {A-18<br>[B-19 | 0.005<br>0.010 | Air.....<br>do.....  | Do.<br>Do.                  |                         |
| 55             | {A-18<br>[C-28 | 0.02<br>1.0    | Air.....<br>Air..... | Poor.<br>Do.                |                         |
| 56             | {A-18<br>[C-26 | 0.02<br>1.0    | Air.....<br>Air..... | Good.<br>Do.                |                         |
| 35             |                | {B-19          | 0.003                | Air.....                    | Do.                     |

## Dispersing agents

Addition of a dispersing agent such as D-1 to the A+B+C combination sometimes improves the rating by increasing the rate of leveling and/or the lustrous current density range. (Examples 51 and 52.)

In other cases, addition of D-1 does not appreciably change the rating but increases the degree of brightness or eliminates microroughness. (Examples 23 and 24.)

## Fluoborate bath

For a fluoborate bath of the preferred composition indicated in Table I, the additives of Example 35 gave equally excellent results. Use of the fluoborate bath allows to increase plating speeds by 50 to 100%.

Although this invention has been illustrated by reference to specific embodiments, modifications thereof which are clearly within the scope of the invention will be apparent to those skilled-in-the-art.

## 55 What is claimed is:

1. A process for electrodepositing bright, strongly leveled, ductile copper from an aqueous acidic copper plating bath containing chloride ions and at least one member independently selected from each of the following groups:

(A) 0.001 g./l. to 1.0 g./l. of a polysulfide compound of the formula



(B) 0.1 mg./l. to 50 mg./l. of a heterocyclic sulfur compound containing the grouping



70 and/or tautomers thereof N-oxides of said compound, isothiourea derivatives, isothioamide derivatives and di-thiocarbamate derivatives thereof; and

(C) 0.005 to 10 g./l. of a polymer containing at least 5 ether oxygen atoms per molecule;



36. An aqueous acidic copper plating bath as claimed in claim 24 wherein the heterocyclic sulfur compound is 6-methyl-2-S-pyridyl isothiouronium chloride N-oxide.

37. An aqueous acidic copper plating bath as claimed in claim 24 wherein the heterocyclic sulfur compound is 2-mercaptopquinoline.

38. An aqueous acidic copper plating bath as claimed in claim 24 wherein the heterocyclic sulfur compound is 2-S-quinolyl isothiouronium chloride.

39. An aqueous acidic copper plating bath as claimed in claim 24 wherein the heterocyclic sulfur compound is 2-mercaptopquinoline N-oxide.

40. An aqueous acidic copper plating bath as claimed in claim 24 wherein the heterocyclic sulfur compound is 2-S-quinolyl isothiouronium chloride N-oxide.

41. An aqueous acidic copper plating bath as claimed in claim 24 wherein the heterocyclic sulfur compound is 2-mercaptop-6-hydroxy pyridine.

42. An aqueous acidic copper plating bath as claimed in claim 24 wherein the heterocyclic sulfur compound is 6-hydroxy-2-S-pyridyl isothiouronium chloride.

43. An aqueous acidic copper plating bath as claimed in claim 24 wherein the heterocyclic sulfur compound is 2,6-dimercapto pyridine.

44. An aqueous acidic copper plating bath as claimed in claim 24 wherein the heterocyclic sulfur compound is 2,6-SS-pyridyl bis-isothiouronium chloride.

45. An aqueous acidic copper plating bath as claimed in claim 24 wherein the heterocyclic sulfur compound is thiocaprolactam (2-thioxohexamethyleneimine).

46. An aqueous acidic copper plating bath as claimed in claim 24 wherein the heterocyclic sulfur compound is 2-S-pyridyl-N-diethyl dithiocarbamate.

#### References Cited

##### UNITED STATES PATENTS

3,542,655 11/1970 Kardos et al. ----- 204—52 R  
3,682,788 8/1972 Kardos et al. ----- 204—52 R

GERALD L. KAPLAN, Primary Examiner

15

20